

March 16, 1937.

F. P. WOOD

2,073,894

PANEL BOARD AND METHOD OF MAKING SAME

Filed Jan. 30, 1936



Inventor:  
Frederick P. Wood,  
By Ranning, Ranning  
Atty's.

## UNITED STATES PATENT OFFICE

2,073,894

PANEL BOARD AND METHOD OF MAKING  
SAMEFrederick P. Wood, Adrian, Mich., assignor to  
Simplex Paper Corporation, Adrian, Mich., a  
corporation of Michigan

Application January 30, 1936, Serial No. 61,505

13 Claims. (Cl. 154—2)

An object of this invention is to provide a panelboard which is relatively hard and stiff and of nearly equal strength in all directions, which is highly water-resistant, and which does not warp, twist, swell or shrink to any appreciable degree under widely different conditions of temperature or humidity.

Another object of this invention is to provide a method of making such a panelboard.

10 Another object of this invention is to provide an improved waterproof asphalt board which is sightly in appearance and particularly adapted for use in the automobile industry, as a panelboard, and the like, and which is economical to manufacture with present equipment.

These and other objects, as will hereinafter appear, are accomplished by this invention which is fully described in the following specification and shown in the accompanying drawing, in

20 which—

Figure 1 is a diagrammatic view showing mechanism for coating a fiber paper which is the first step in making the panelboard;

Fig. 2 is a greatly enlarged transverse section 25 through a sheet of fiber paper coated by the apparatus of Fig. 1;

Fig. 3 is a diagram of mechanism for assembling two such sheets of fiber paper to make the panelboard;

30 Fig. 4 is a greatly enlarged transverse section of a sheet of panelboard made by the apparatus of Fig. 3; and

Fig. 5 is a partial side elevation of a truck for compressing and holding a stack of sheets of 35 such panelboard during the setting operation.

This is a continuation in part of my applications for patent Serial No. 591,520, filed February 8, 1932, and Serial No. 21,762, filed May 16, 1935.

Generally speaking, the panelboard is composed of two, three, four or more sheets of paper each of a thickness of .016" or more (preferably .0026" or .0032" which I am now using, or more) of a kraft pulp or the like. This is so made that the fibers of the paper which are nearly pure

45 cellulose, are running nearly equally in all directions, each sheet being separately treated to render it water-resistant, and the sheets assembled with a suitable adhesive between them. For this purpose the paper may be made of 50 kraft sulphate pulp or other chemical pulp, or fiber on a Fourdrinier paper machine. Paper so made possesses a strength and rigidity in a direction across the grain of two-thirds or more of the strength with the grain, (i. e., the direction of travel of the sheet through the paper

5 machine) because the fibers are arranged in the paper nearly equally in all directions due to the rotary vibratory motion of the pulp collecting mechanism while the pulp is being formed into sheets.

This pulp paper is sized, preferably in the beater, with a suitable size, such as a soluble resin soap, alum being added to change the soluble soap into an insoluble soap in a well known manner. This soap is precipitated on the sides and 10 ends of the individual cellulose fibers, while still in the beater, by the addition of an acid. The amount of size added is sufficient to make the paper "hard sized". In this condition, the resulting paper is water-resistant but will not resist 15 expansion or contraction under varying moisture conditions. If the kraft paper is not properly sized, the panelboard made from it, as will later be explained, will absorb too much water.

This kraft pulp paper has one essential for this 20 purpose, i. e., it is a single layer of fibers, whereas in a paper made on a cylinder machine, there are as many layers as there are cylinders in use, the fibers of one layer being discontinuous from the fibers of the next adjacent layer. Consequently the hot liquid filler, as asphalt or resin, 25 is able to penetrate from one layer to the next but slowly in the case of the paper made on the cylinder machine, whereas it penetrates rapidly into the kraft paper because the fibers are continuous, and are relatively long.

In Fig. 1 is shown a mechanism for treating 30 a single sheet of pulp paper for this purpose with a suitable waterproofing material. In this mechanism the sheet of pulp paper to be treated is 35 unwound from a reel A, passes over steam-heated rolls 11 and down under rollers 13 and 14 in a tank 15 so as to pass beneath the surface of molten asphalt 16 which is preferably heated in any well known manner, as by a furnace thereunder, 40 at a temperature of about 400° to 425° F. Air and water in the paper are expelled and are carried off by the pipe 12 which leads to a stack. The tank has sliding covers 15a.

This tank is sufficiently long to give the molten 45 asphalt time to penetrate well into the fiber of the paper which preferably is traveling 180 to 225' per minute. For some purposes, the paper may be saturated throughout by the asphalt, while for other purposes it is preferable that the 50 paper will not be saturated all the way through, but instead will leave a central unsaturated or semi-saturated core, as shown in Fig. 2. I preferably use an asphalt which is very hard and brittle having a melting point of not less than 55

140° F. and having a penetration point of not over 22, as expressed in units of the American Society for Testing Materials, designation D5—25, which is the standard method of test for penetration 5 for bituminous materials. According to the description of this test, the result 22 in this case is expressed in degrees, each degree being equivalent to 1/100th of a centimeter, which a standard needle will vertically penetrate a sample of the 10 material in five seconds under a load of 100 grams, the material being at a temperature of 77° F.

When the paper treated in this way leaves the tank of asphalt, it is nearly free from water, is 15 brittle, and is preshrunk and it passes out between two pressure rolls 17, where it is squeezed fairly dry of excess asphalt. Enough asphalt remains, however, to make the surface of the 20 sheet very shiny as it leaves the squeezing rolls. 25 If this sheet is held in the air for a few seconds, this surface asphalt is rapidly drawn into the sheet. I accordingly place rolls 18, 19 some distance from the rolls 17 so as to provide a stretch 30 long enough for this absorption to take place. 35 The paper is then cooled by the water-cooled rolls 18, 19 and is wound up on a roll B. This paper is bone dry and avid for moisture which must be added to it in some way in order to restore the necessary toughness to the sheet. If 30 left in the air for some time, it will absorb 7% to 8% of its weight in moisture but will take it up in the roll but slowly through the edges.

To make a panelboard, two or more sheets of 35 this pulp are then secured together with a suitable waterproof adhesive between them, as many sheets as desired being used to make any desired thickness of board. The adhesive used contains sufficient water to give the panelboard a normal moisture content of 7% to 8%, thereby returning 40 the toughness to the paper. This water is absorbed by the board even when asphalt has passed all the way through.

To make this panelboard, two such rolls of 45 paper B', B<sup>2</sup> are mounted in the mechanism shown in Fig. 3. The sheet from B' is led over a roller 23 between rollers 24, 25, the latter dipping into a bath of a suitable waterproof adhesive 26. For this purpose I prefer to use a cement composed of nearly equal parts of rubber latex 50 and starch paste containing water as a solvent. The starch has the jelling properties removed but is not dextrinized. Less rubber may be used if desired. Ammonia present in the rubber latex keeps it in a state of emulsion. 2% to 3% of a 55 soft asphalt emulsified with silicate of soda, clay, etc., adds greatly to the strength of the cement. The sheet so coated with cement is brought into juxtaposition with the sheet from the roll B<sup>2</sup> and the two sheets are firmly pressed together as they 60 pass through between pressing rolls 27, after which they are preferably passed through cutters 28 which cut the sheet 29 into panelboard rectangles 29<sup>a</sup> which are preferably stacked on a truck 30. A top plate or cover 31 is placed on 65 top of the pile and clamped down by means of tightening screws 32 and nuts 33.

When the sheet emerging from the asphalt bath 16 passes the squeezing rollers 17, it may be completely saturated with asphalt or it may 70 possess a cross section like that shown in Fig. 2 in which there may be an unsaturated or semi-saturated central core 50 with infiltration layers 41, 42 of hard asphalt. The fibers of the sheet assembled as they are on a Fourdrinier machine 75 run in all directions and many of the fibers 43

extend from points outside the asphalt to points well within the asphalt. When the sheet emerges from the bath of asphalt, the heat of the asphalt has expelled substantially all of its moisture, so that the sheet emerges in a very dry state.

When the waterproof starch adhesive is applied, it preferably contains just sufficient water to return the fiber sheet to a normal moisture content. The protruding fiber ends 43 are buried in the waterproof starch adhesive 26 (Fig. 4) 10 and hence in intimate contact therewith, and it is my theory that moisture, probably because of the partial sealing effect of the asphalt, and resin 15 size passes very slowly along or through these fibers by capillary attraction, and as it does so carries with it the waterproof starch adhesive. This is possible because of the fact that the water and air normally within the cells of the fibers themselves has been expelled by the heat treatment so that the voids thus created permit the 20 water to be sucked in. The result is that the adhesive is drawn well into the body of the sheet along or through these fibers as through minute tubes, and as it slowly sets firmly cements the 25 two sheets together. The rubber latex then serves to exclude moisture so that even though the panelboard is placed in water for a considerable period of time after it has once set, very little softening of the adhesive takes place. In 30 addition, the latex adds some adhesive action. An adhesive such as casein and lime, albumen and lime, or any other water-soluble adhesive containing some waterproofing agent may be used instead of the latex starch mixture, but most of 35 these are more costly.

When the sheets 29 are first assembled the cement has not yet had time to set, consequently the sheets composing the panelboard can be readily separated. After it has been held clamped on the truck for a period of four to six hours, 40 the cement becomes thoroughly set and the sheets can no longer be separated on the central plane. This panelboard can be readily pressed into various shapes just after it emerges from the cutters 45 29 and before it has had time to set. After pressing, it should be left in the desired form until the cement has set, as previously explained, after which it will retain that form. By raising this moisture content to 10-12% the panelboard can be kept in a moist room for months before pressing. On pressing, it dries and sets as before.

For certain purposes the central core may be practically saturated with asphalt and still take up very considerable quantities of moisture from the cement so as to be quite tough because of 55 a return thereto of a normal moisture content.

When panelboards are thus made they have a normal moisture content of 7-8% by weight so that these panels can be taken into regions having very widely different humidity without any tendency of the panelboard to shrink, expand, warp, buckle or cockle even when the panelboard is 60 immersed in water for several hours or subjected to very dry atmosphere for long periods.

It is found in practice that a much harder asphalt may be used to advantage. For example, an asphalt having a melting point of 160° F. and a penetration point of 4 has proved highly satisfactory. The limits set out earlier are intended to mark approximately the softer limits of asphalt for good results in the panelboard.

In actual practice, this panelboard has been found to possess unusual strength and rigidity in all directions, to be highly water-resistant, and to be little affected by changes of temperature 75

and humidity, so that it is particularly suited for use as a panelboard for automobiles, and the like. For such a purpose this board can be cut and punched to size, and in this condition can be

5 shipped over long distances and stored for long periods and later assembled without the danger that it will not fit the parts with which it was intended to be assembled.

This panelboard has a surface which readily 10 adapts it to painting, embossing in imitation of leather, and the like, directly thereon, or cloth trim may be secured thereon by means of a suitable adhesive without danger of warping or of the asphalt coming through the cloth, since it is 15 my theory that the asphalt is trapped and held within the interstices between the fibers, so that the hard and brittle asphalt becomes, as it were, a permanent constituent of the structure of the panelboard and will not exude or release therefrom under any conditions encountered in service.

For certain purposes, the hard asphalt may be 20 replaced by a hard brittle resin, or coal tar pitch, or wood pitches, either natural or synthetic, which is applied molten in the same way as the asphalt. The resulting panelboard will take the same adhesive as for asphalt and will be moisture-proof in about the same degree. The cost is considerably more. The resin filled sheet may be 25 given any desired color, or it may be printed to resemble a wood grain. The outer layer may be thus treated while the other layers are filled with asphalt.

While I prefer to use a beater sized pulp sheet, 30 it may, if desired, be tub sized. Paraffin may also be used as a tub size after which the sheet is treated with molten paraffin or resin as before.

For the sake of illustration, I have shown 35 two sheets of pulp, but in actual practice, I find it advantageous to use three sheets and apply 40 the cement to both sides of the central sheet, the two uncoated outer sheets then being pressed into contact with the central sheet. For certain purposes, I also precut the sheets and turn one sheet so that its grain runs at right angles to 45 that of another sheet.

The ends of the fibers protruding beyond the 50 surface of the panelboard may be noticeable and, if desired, these may be dyed any color as by means of an alcohol soluble dye. The outer 55 surface may also be coated with a waterproof material, such as tung oil, to further assist in special cases in preventing the ingress and egress of moisture.

I claim:

55 1. A product in sheet form which is highly resistant to physical change in a wide range of temperature and humidity conditions, comprising a sheet of sized fibre pulp consisting of a singly formed layer of fibres of nearly pure cellulose disposed substantially uniformly in all directions, said sheet being partially impregnated with asphalt having a melting point of not less than 140° F. and a penetration point of not over 22, the surface fibres of the sheet exceeding beyond the body of asphalt, whereby 60 said sheet may be cemented to an adjacent surface.

2. A panelboard comprising two superposed 65 sheets, at least one of said sheets being resistant to physical change in a wide range of temperature and humidity conditions, said sheet being composed of sized fibre pulp consisting of a singly formed layer of fibres of nearly pure cellulose disposed substantially uniformly in all 70 directions, said sheet being impregnated with

asphalt having a melting point of not less than 140° F. and a penetration point of not over 22, and an adhesive uniting the surface fibres of the superposed sheets.

3. A panelboard comprising two superposed 5 sheets, each sheet being resistant to physical change in a wide range of temperature and humidity conditions, each sheet being composed of sized fibre pulp consisting of a singly formed layer of fibres of nearly pure cellulose disposed substantially uniformly in all directions, each sheet being impregnated with asphalt having a melting point of not less than 140° F. and a penetration point of not over 22, the surfaces of the sheets having protruding fibres, and an 10 adhesive uniting adjacent surfaces of the sheets, said adhesive extending into the body of the 15 sheets through said protruding surface fibres.

4. A panelboard comprising two superposed 20 sheets, each sheet being resistant to physical change in a wide range of temperature and humidity conditions, each sheet being composed of sized fibre pulp consisting of a singly formed layer of fibres of nearly pure cellulose disposed substantially uniformly in all directions, each sheet being impregnated with asphalt having a melting point of not less than 140° and a penetration point of not over 22, the surfaces of the 25 sheets having protruding fibres, and a waterproof starch adhesive uniting adjacent surfaces 30 of the sheets, the starch of said adhesive extending into the body of the sheets through said protruding surface fibres.

5. The method of making a product in sheet 35 form which is highly resistant to physical change in a wide range of temperature and humidity conditions which comprises impregnating a sheet of sized fibre pulp with molten asphalt, then simultaneously compressing the fibres of the sheet and removing the excess asphalt therefrom, then allowing the fibres of the sheet to expand for a predetermined period of time to draw the surface layers of asphalt into the body 40 of the sheet and cooling the sheet.

6. The method of making a product in sheet 45 form which is highly resistant to physical change in a wide range of temperature and humidity conditions which comprises passing a sheet of sized fibre pulp through a bath of molten, hard and brittle asphalt for a period of time 50 sufficient to simultaneously impregnate the sheet and remove substantially the entire normal moisture content of the sheet, then passing the sheet between squeezing rolls to simultaneously compress the fibres of the sheet and remove 55 excess asphalt therefrom, then allowing the fibres of the sheet to expand and the sheet to cool for a predetermined period of time to draw the molten asphalt into the body of the sheet, and then finally adding sufficient moisture to 60 the sheet to restore its normal moisture content.

7. The method of making a product in sheet 65 form which is highly resistant to physical change in a wide range of temperature and humidity conditions which comprises passing a sheet of sized fibre pulp through a bath of molten, hard and brittle asphalt for a period of time sufficient to simultaneously impregnate the sheet and remove substantially the entire normal moisture content of the sheet, then passing 70 the sheet between squeezing rolls to simultaneously compress the fibres of the sheet and remove excess asphalt therefrom, then allowing the fibres of the sheet to expand and the sheet to cool for a predetermined period of time to 75

- draw the molten asphalt into the body of the sheet, applying an adhesive containing water to one surface of the dehydrated sheet, said water also restoring the normal moisture content to the dehydrated sheet, bringing a second sheet into contact with the adhesive layer on the first sheet, and finally pressing the sheets together.
8. The method of making a product in sheet form which is highly resistant to physical change in a wide range of temperature and humidity conditions which comprises impregnating a sheet of sized fibre pulp having the fibres disposed nearly uniformly in all directions with molten asphalt having a melting point of not less than 140° F. and a penetration point of not over 22 at a temperature and for a period of time sufficient to dehydrate the sheet, simultaneously compressing the fibres of the sheet and removing the excess asphalt therefrom as the sheet leaves the molten asphalt, and suspending the sheet in the air for a predetermined period to permit the sheet to draw the molten surface asphalt into the body of the sheet.
9. The method of making a product in sheet form which is highly resistant to physical change in a wide range of temperature and humidity conditions which comprises impregnating a sheet of sized fibre pulp having the fibres disposed nearly uniformly in all directions with molten asphalt having a melting point of not less than 140° F. and a penetration point of not over 22 at a temperature and for a period of time sufficient to dehydrate the sheet, simultaneously compressing the fibres of the sheet and removing the excess asphalt therefrom as the sheet leaves the molten asphalt, suspending the sheet in the air for a predetermined period to permit the sheet to draw the molten surface asphalt into the body of the sheet, and then cooling the sheet.
10. The method of making a product in sheet form which is highly resistant to physical change in a wide range of temperature and humidity conditions which comprises impregnating a sheet of sized fibre pulp having the fibres disposed nearly uniformly in all directions with molten asphalt having a melting point of not less than 140° F. and a penetration point of not over 22 at a temperature and for a period of time sufficient to dehydrate the sheet, simultaneously compressing the fibres of the sheet and removing the excess asphalt therefrom as the sheet leaves the molten asphalt, suspending the sheet in the air for a predetermined period to permit the sheet to draw the molten surface asphalt into the body of the sheet, and adding sufficient moisture to the sheet to restore its normal moisture content.
11. The method of making a product in sheet form which is highly resistant to physical change in a wide range of temperature and humidity conditions which comprises impregnating a sheet of sized fibre pulp having the fibres disposed nearly uniformly in all directions with molten asphalt having a melting point of not less than 140° F. and a penetration point of not over 22 at a temperature and for a period of time sufficient to dehydrate the sheet, simultaneously compressing the fibres of the sheet and removing the excess asphalt therefrom as the sheet leaves the molten asphalt, suspending the sheet in the air for a predetermined period to permit the sheet to draw the molten surface asphalt into the body of the sheet, applying an adhesive containing water to one surface of the sheet to restore the normal moisture content to said sheet, and bringing a second sheet into intimate contact with the adhesive on the first sheet.
12. The method of making a product in sheet form which is highly resistant to physical change in a wide range of temperature and humidity conditions which comprises impregnating a sheet of sized fibre pulp having the fibres disposed nearly uniformly in all directions with molten asphalt having a melting point of not less than 140° F. and a penetration point of not over 22 at a temperature and for a period of time sufficient to dehydrate the sheet, simultaneously compressing the fibres of the sheet and removing the excess asphalt therefrom as the sheet leaves the molten asphalt, suspending the sheet in the air for a predetermined period to permit the sheet to draw the molten surface asphalt into the body of the sheet, applying an adhesive containing water to one surface of the sheet, bringing a second sheet into contact with the adhesive on the first sheet, pressing the sheets together, and applying pressure to the sheets until the adhesive sets.
13. The method of making a product in sheet form which is highly resistant to physical change in a wide range of temperature and humidity conditions which comprises impregnating a sheet of fiber pulp in a bath of molten material which renders the sheet water-resistant, said impregnating being done at a temperature and for a period of time sufficient to remove substantially all the moisture from the sheet, removing the excess molten material, applying an adhesive containing water to one surface of the dehydrated sheet, said water also restoring the normal moisture content of the dehydrated sheet, bringing a second sheet into contact with the adhesive layer on the first sheet, and pressing the sheets together.

FREDERICK P. WOOD.